

# United States Patent [19]

Takemura

[11] 3,876,421

[45] Apr. 8, 1975

- [54] **PROCESS FOR DESULFURIZATION OF MOLTEN PIG IRON**
- [75] Inventor: **Yozo Takemura, Tokai, Japan**
- [73] Assignee: **Nippon Steel Corporation, Tokyo, Japan**
- [22] Filed: **Nov. 5, 1973**
- [21] Appl. No.: **412,766**

|           |         |                 |       |
|-----------|---------|-----------------|-------|
| 2,863,755 | 12/1958 | Kurzinski ..... | 75/58 |
| 2,870,004 | 1/1959  | Estes .....     | 75/51 |
| 2,979,393 | 4/1961  | Hever .....     | 75/51 |
| 3,158,913 | 12/1964 | Bolkcom .....   | 75/58 |
| 3,350,196 | 10/1967 | Bashford .....  | 75/52 |
| 3,473,917 | 10/1969 | Michaelis ..... | 75/52 |
| 3,556,773 | 1/1971  | Grenfell .....  | 75/52 |
| 3,622,302 | 11/1971 | Hayashi .....   | 75/58 |
| 3,704,230 | 11/1972 | Loricchio ..... | 75/58 |
| 3,768,999 | 10/1973 | Ohkubo .....    | 75/58 |

[30] **Foreign Application Priority Data**

Nov. 9, 1972 Japan .....

47-111636

Feb. 23, 1973 Japan .....

48-21866

[52] **U.S. Cl. .... 75/58; 75/51; 75/53**

[51] **Int. Cl. .... C21c 7/02**

[58] **Field of Search .....** 75/53-60, 51,  
75/52

[56] **References Cited**

UNITED STATES PATENTS

2,577,764 12/1951 Hulme .....

*Primary Examiner*—L. Dewayne Rutledge

*Assistant Examiner*—Peter D. Rosenberg

*Attorney, Agent, or Firm*—Toren, McGeady and  
Stanger

[57] **ABSTRACT**

A process for desulfurization of molten pig iron, which comprises mixing calcium carbide with a gas generating substance and adding the mixture into the molten pig iron with a carrier gas.

**5 Claims, 3 Drawing Figures**

SHEET 1 OF 2

F I G. 1



F I G. 2

CARBIDE +15% COKE POWDER +85% LIME STONE.

BEFORE TREATMENT

AFTER TREATMENT

S: 0.03% → S: 0.01%



FIG. 3



# PROCESS FOR DESULFURIZATION OF MOLTEN PIG IRON

The present invention relates to a process for desulfurization of molten pig iron.

In the conventional process for desulfurization of molten pig iron, calcium carbide has been hitherto added. The desulfurization shows a reaction efficiency of 5 to 15 percent when it is added through a carrier gas and of 20 to 25 percent when it is mechanically agitated for desulfurization, for example, by an impeller. Thus, the reaction efficiency is particularly low with carrier gas.

The present invention provides an excellent method to improve the efficiency when a carrier gas is used and is characterized by (1) a process for desulfurization of molten pig iron in which calcium carbide having a particle size of about 10 mm or less is mixed with a gas generating substance and added to the molten pig iron through a carrier gas; (2) a process for desulfurization of molten pig iron, in which carbide is mixed with a gas generating substance and added to the molten pig iron through a carrier gas, having a reducing gas therein; (3) a process for desulfurization of molten pig iron, in which a granulated desulfurizing agent, made of carbide mixed with a gas generating substance is added to the molten pig iron; (4) a process for desulfurization of molten pig iron, in which petroleum substances are added to the molten pig iron to promote the desulfurization; and (5) a desulfurizing agent for molten pig iron composed of calcium carbide mixed with a gas generating substance, in which 10 to 50 percent of said carbide is admixed with a foaming gas.

The present invention shall be explained in detail, referring to the drawings, in which

FIG. 1 is a diagram, showing the relation of the size of the desulfurizing agent (carbide) to the desulfurization effect;

FIG. 2 is a diagram, showing the relation of the size of the sulfurizing agent and the ratio of mixing in the carrier gas (including the gas generating substance) to the desulfurization efficiency; and

FIG. 3 is a diagram showing the relation between the ratio of the desulfurizing agent, mixed with the carrier gas (foaming gas) and the desulfurization efficiency.

According to the result of various investigations made by the present inventors on the relation between the desulfurization reaction and the desulfurizing agent (carbide), as shown in FIG. 1, carbide having a particle size of 0.5 to 1.1 mm shows the increase of the desulfurization efficiency, but it is not possible to improve the desulfurization efficiency when sizes different from those shown in the drawing are used. For particle sizes of about 1.1 mm or above, the surface of the desulfurizing agent becomes small and the area to be contacted with molten pig iron becomes small, so that it is natural that the desulfurization efficiency is decreased. Though it is a common-sense view that if the size becomes about 0.5 mm or below, the desulfurization effect is improved by the large area per unit weight of contact with the molten pig iron, the efficiency is decreased as shown in the drawing when the size of the desulfurizing agent becomes about 0.5 mm or below. We have found that it is due to the following reason:

When the desulfurizing agent is blown (added) into the molten pig iron through a carrier gas, it is desirable to introduce the agent in the bottom part of the vessel

in order to increase the efficiency by elongation of the contact time with the molten pig iron. The time depends upon the capacity of the vessel, but it generally takes about 1.0 sec. for the foam of carrier gas to be

5 floated from the point at which it is blown in to the surface of the molten pig iron. It is necessary that the desulfurizing agent, blown in through the carrier gas, is sufficiently contacted with the molten pig iron during this time. However, a large amount of the desulfurizing agent, blown in through the carrier gas enters, enter into the foam of the carrier gas and some of the desulfurizing agents in the foam reach the peripheral part of the foam under their own weight in the process of floating toward the surface of the molten pig iron, while the 10 others remain in the foam and continue to be floated up. Therefore, the desulfurizing agent for contact with the molten pig iron diminishes, so that the desulfurization efficiency is decreased.

That is to say, particle size range which enables the 15 movement of the agent toward the periphery of the foam by its own weight, is 0.5 to 1.1 mm. If the size is about 0.5 mm or below, the agent floats in the foam and comes to the surface of the molten pig iron without contacting the molten pig iron. Consequently, the desulfurization efficiency can be significantly increased if the floating foam is broken and the desulfurizing agent in the foam is fully contacted with the molten pig iron.

Therefore, the desulfurizing agent is mixed with a foam breaking substance. For example, a substance 20 which generates gas when treated and is added i.e., blown into in the molten pig iron through a carrier gas, whereby gas can be generated in the molten pig iron from the gas generating substance contained in the foam, and the foam may be expanded and thus broken 25 (exploded), so that the desulfurizing agent, contained in the foam is fully contacted with the molten pig iron to increase the desulfurization efficiency. For the gas generating substance, a reducing agent, for example, petroleum substances, such as heavy oil, tar or the like, 30 cokes, Al powders or polyester, are mixed in a  $\text{CO}_2$  gas generating substance, such as, limestone or  $\text{MgCO}_3$  to convert  $\text{CO}_2$  to  $\text{CO}$  (a reducing gas). Thus, oxidation of the surface of the desulfurizing agent can be prevented by  $\text{CO}_2$  so that the desulfurization efficiency can 35 be increased. The quantity to be added in the desulfurizing agent is 7 to 20 percent. To break the foam, a mixing ratio with the carrier gas as explained below is used. The mixture of the desulfurizing agent and the gas generating substance can sufficiently break the foam in the 40 molten pig iron when the mixing ratio with the carrier gas, i.e.:

$$\frac{\text{Quantity of } \text{CO}_2 \text{ generated from the desulfurizing agent/min.}}{\text{Quantity of carrier gas/min.}} \times 100$$

55 is from 10 to 50 percent. If the quantity (ratio) of the gas generating substance to be added in the desulfurizing agent is about 7 percent or below, the quantity of 60 gas generated is not enough. It can scarcely expand the foam and sometimes it becomes impossible to break the foam. If the ratio is about 20 percent or above, the flame or boiling becomes vehement and the operation become dangerous. Accordingly, when the amount of 65 gas generating substance is 20 percent, the ratio of the carrier gas mixed with the gas generating substance, including the desulfurizing agent, is about 50 percent or

below in order to break the foam fully. The desulfurization efficiency can be increased as shown in FIG. 2, when the mixing ratio with the carrier gas is about 10 percent or above. Moreover, according to the present invention, the desulfurization can be efficiently performed by adding the desulfurizing agent through the carrier gas. Such excellent desulfurization effects can be brought about easily and simply.

The relation of the mixing ratio of the desulfurizing agent and the carrier gas (foaming gas) to the desulfurization efficiency is shown in FIG. 3.

If such a gas generating substance is mixed to generate gas in the molten pig iron, carbide is oxidized by  $\text{CO}_2$  gas in the reaction:  $\text{CaC}_2 + \text{CO}_2 \rightarrow \text{CaO} + \text{CO}$  and becomes less active for the desulfurization reaction. The desulfurization efficiency thus is sometimes decreased.

In this case, if a reducing gas, such as,  $\text{H}_2$ ,  $\text{CH}_4$ ,  $\text{C}_2\text{H}_4$  or  $\text{C}_3\text{H}_8$  is contained in the carrier gas and the carbide, mixed with the beforementioned gas generating substance is carried in the molten pig iron,  $\text{CO}_2$  generated in the molten pig iron is reduced in the reaction of  $\text{CO}_2 + \text{reducing gas} \rightarrow \text{CO}$ . The carbide can be prevented from the surface oxidization of  $\text{CO}_2$  gas. The surface of carbide, dispersed in the molten pig iron by the breaking of the foam, can be contacted with the molten pig iron in the active condition, so that the desulfurization reaction may be significantly improved. If the reducing gas is used in this manner according to the present invention, the reaction of  $\text{CO}_2 + \text{reduction} \rightarrow \text{CO}$  is instantaneously carried out as compared with the case of a solid substance, such as C, used as the reducing agent. Therefore, carbide is almost not oxidized and the desulfurization effect can be largely improved.

Further, the present inventors have found that when calcium carbide, a desulfurizing agent, is granulated after mixing with a gas generating substance and added to the molten pig iron, gas is generated by the heat of the molten pig iron to pulverize or explode the desulfurizing agent in the molten pig iron, whereby the area of the desulfurizing agent, contacted with the molten pig iron is increased, so that the desulfurization efficiency can be improved.

Further, the present inventors have learned that when carbide is added through the carrier gas, the carbide, blown in the molten pig iron, is confined in the bubble of the carrier gas and often comes to the surface of the molten pig iron without taking part in the desul-

furization reaction, so that the yield of the desulfurizing agent is sometimes decreased.

The present inventors have found that in order to eliminate such a difficulty advantageously, a process, in which petroleum substances are added with carbide into the molten pig iron, is favourable in the case of carbide being added to the molten pig iron for desulfurization.

For the petroleum substance to be used according to 10 the present invention, any such substance in the form of a gas, liquid and solids will do. Gases, such as, propane, butane liquids, such as, heavy oil, tar, kerosene, naphtha, solids, and such as, polyethylene, and vinyl chloride may be used.

15 When a solid is used, it is divided into fine particles of about 0.1 mm or below and mixed with carbide so that the desulfurization effect can be improved.

It seems that the petroleum substance has C and H as the main ingredient and when it is added in molten pig iron, a cracked gas ( $\text{H}_2$ ) is first generated at the temperature, whereby the oxide film is peeled from the carbide to expose the surface, which possesses a high activity and this surface is contacted with the molten pig iron to improve the desulfurization effect.

20 25 The carbide is covered with the cracked gas ( $\text{H}_2$ ) to interrupt the reaction of  $\text{N}_2$ ,  $\text{O}_2$  and carbide, so that the change of  $\text{CaC}_2 \rightarrow \text{CaO}$  and  $\text{CaCN}_2$  does not occur. Further, when it is added in the molten pig iron through the carrier gas, the foam is broken by the cracked gas ( $\text{H}_2$ ) of the petroleum substance and the carbide, contained in the foam, is contacted with the molten pig iron to react, whereby the desulfurization effect can be improved.

30 35 Accordingly, the quantity of petroleum substance to be added may be so determined as to be 0.04 to 1.0 percent, computed on the basis of the quantity of  $\text{H}_2$  gas to be generated

Quantity of  $\text{H}_2$ , generated from the petroleum substance Kg

40 45 Quantity of carbide Kg  
whereby the desulfurization efficiency can be advantageously increased.

If it is less than about 0.04 percent, the quantity of  $\text{H}_2$  gas (cracked gas) generated is very small and the improved effect will not be obtained. If it is about 1.0 percent or above, the cracked gas ( $\text{H}_2$ ) is increased, and flaming and boiling becomes vehement, and is dangerous.

Examples of the inventive process are as follows:

| Inventive examples | Desulfurizing agent | Size of desulfurizing agent | Ratio of gas generating substance to reducing agent | Ratio to carrier gas (mixing ratio) |
|--------------------|---------------------|-----------------------------|-----------------------------------------------------|-------------------------------------|
| 1                  | calcium carbide     | 0.5 mm                      | coke 7%<br>10                                       | $\text{CaCO}_3$ 93%<br>90 20        |
| 2                  | "                   | 1.0                         |                                                     | Al                                  |
| 3                  | "                   | 0.3                         | 15 5                                                | 80                                  |
| 4                  | "                   | 0.1                         | 20 10                                               | 70 30                               |
| 5                  | "                   | 0.1                         | poly-ester<br>10                                    | lime<br>stone<br>90 25              |
| 6                  | "                   | 0.05                        | heavy oil<br>10                                     | raw dolomite<br>90 45               |

  

| Comparative examples |   |     |
|----------------------|---|-----|
| 1                    | " | 0.5 |
| 2                    | " | 1.0 |
| 3                    | " | 0.3 |
| 4                    | " | 0.1 |

| Quantity of desulfurizing agent to be added in molten pig iron a6 | Rate of desulfurizing agent to be added in molten pig iron | Sulphur in molten pig iron before desulfurization | Sulfur in molten pig iron after desulfurization | Reaction efficiency | Inventive examples      | Desulfurizing agent | Size of desulfurizing agent | Ratio of mixing in gas generating substance and carbide | Carrier gas    |
|-------------------------------------------------------------------|------------------------------------------------------------|---------------------------------------------------|-------------------------------------------------|---------------------|-------------------------|---------------------|-----------------------------|---------------------------------------------------------|----------------|
| kg/t-pig                                                          | kg/t-min.                                                  | %                                                 | %                                               | %                   |                         |                     |                             |                                                         |                |
| 2.5                                                               | 0.1                                                        | 0.03                                              | 0.01                                            | 19                  | 8                       | calcium carbide     | 0.5 mm                      | CaCO <sub>3</sub> : 15 %                                | N <sub>2</sub> |
| 2.6                                                               | 0.2                                                        | 0.04                                              | 0.015                                           | 23                  | 9                       | "                   | 1.0                         | MgCO <sub>3</sub> : 10                                  | "              |
| 4.1                                                               | 0.3                                                        | "                                                 | 0.005                                           | 20                  |                         | "                   | 0.3                         | CaCO <sub>3</sub> : 10                                  | Ar             |
| 1.5                                                               | 0.06                                                       | "                                                 | 0.02                                            | 30                  | 10                      | "                   | 0.1                         | MgCO <sub>3</sub> : 10                                  |                |
| 1.0                                                               | 0.5                                                        | 0.03                                              | 0.01                                            | 40                  |                         |                     |                             | CaCO <sub>3</sub> : 10                                  | N <sub>2</sub> |
| 1.2                                                               | 0.2                                                        | 0.04                                              | 0.015                                           | 32                  | 10 Comparative examples |                     |                             |                                                         |                |
| 4.7                                                               | 0.15                                                       | 0.03                                              | 0.01                                            | 10                  |                         |                     |                             |                                                         |                |
| 4.7                                                               | 0.3                                                        | 0.04                                              | 0.015                                           | 12                  |                         | 5                   | "                           | carbide singly                                          | N <sub>2</sub> |
| 11.8                                                              | 0.3                                                        | "                                                 | 0.005                                           | 7                   |                         | 6                   | "                           | "                                                       | Ar             |
| 9.5                                                               | 0.33                                                       | "                                                 | 0.02                                            | 5                   |                         | 7                   | "                           | 1.0                                                     | N <sub>2</sub> |
|                                                                   |                                                            |                                                   |                                                 |                     |                         | 8                   | "                           | 0.3                                                     |                |
|                                                                   |                                                            |                                                   |                                                 |                     |                         |                     |                             | CaCO <sub>3</sub> : 15                                  |                |
|                                                                   |                                                            |                                                   |                                                 |                     |                         |                     |                             | MgCO <sub>3</sub> : 10                                  | "              |

Note 1:

The molten pig iron of 1200°C was filled in a ladle and blown in under the surface of molten pig iron.

15

Note 2:

The ratio to carrier gas is the volumetric ratio of the mixture of a desulfurizing agent and a gas generating substance, thrown in the carrier gas:

Quantity of CO gas, generated from the gas generating substance/min.

Quantity of carrier gas/min. × 100

Note 3:

The reaction efficiency is:

Quantity of CaC<sub>2</sub>, taking part in the desulfurization reaction  
Quantity of CaC<sub>2</sub> to be added × 100

| Ratio of addition in reducing gas and carrier gas | Desulfurization reaction |                         | Unit of desulfurizing agent | Reaction efficiency |
|---------------------------------------------------|--------------------------|-------------------------|-----------------------------|---------------------|
|                                                   | S before desulfurization | S after desulfurization |                             |                     |
| CH <sub>4</sub> : 10 %                            | 0.03                     | 0.01                    | 2.0 kg/t-pig                | 26.5 %              |
| C <sub>2</sub> H <sub>6</sub> : 5                 | 0.05                     | 0.015                   | 3.0                         | 31.5                |
| C <sub>3</sub> H <sub>8</sub> : 3                 | 0.03                     | 0.01                    | 1.5                         | 35.5                |
| " : 3                                             | 0.05                     | 0.015                   | 2.7                         | 34.5                |
|                                                   | 0.03                     | 0.01                    | 4.5                         | 11.8                |
|                                                   | 0.05                     | 0.015                   | 6.0                         | 15.5                |
|                                                   | 0.03                     | 0.01                    | 5.5                         | 9.7                 |
|                                                   | 0.05                     | 0.015                   | 8.0                         | 11.6                |

Note :

The molten pig iron of 1200°C was filled in a ladle and blown in under the surface of molten pig iron.

| Inventive examples | Size of calcium carbide | Gas generating substance | Ratio of gas generating substance, added to carbide | Size of gas generating substance after addition |
|--------------------|-------------------------|--------------------------|-----------------------------------------------------|-------------------------------------------------|
|--------------------|-------------------------|--------------------------|-----------------------------------------------------|-------------------------------------------------|

|    |               |                                                   |     |          |
|----|---------------|---------------------------------------------------|-----|----------|
| 11 | below 0.2 mm  | lime stone + C<br>85% + 15%<br>tar + C<br>80 + 20 | 10% | 1 ~ 2 mm |
| 12 | "             | lime stone<br>100                                 | 5   | 2 ~ 3    |
| 13 | below 0.05 mm | lime stone<br>100                                 | 30  | 1 ~ 2    |
| 14 | below 0.2 mm  | polyester<br>100                                  | 5   | 1 ~ 3    |

Comparative examples

9 0.2 to 1.0 mm  
10 below 0.2 mm  
11 "  
12 0.2 to 1.0 mm

| Quantity of desulfurizing agent | Sulphur in molten pig iron before desulfurization | Sulphur in molten pig iron after desulfurization | Reaction efficiency |    |
|---------------------------------|---------------------------------------------------|--------------------------------------------------|---------------------|----|
| 1.5 kg/t-pig                    | 0.03 %                                            | 0.016                                            | 25 %                |    |
| 2.0                             | 0.04                                              | 0.017                                            | 30                  | 5  |
| 2.5                             | "                                                 | 0.008                                            | 35                  |    |
| "                               | "                                                 | 0.008                                            | "                   |    |
| 2.7                             | 0.03                                              | 0.015                                            | 15                  |    |
| 2.5                             | 0.04                                              | 0.033                                            | 7                   |    |
| "                               | "                                                 | 0.023                                            | 6                   |    |
| 3.0                             | "                                                 | 0.015                                            | 13                  |    |
|                                 |                                                   |                                                  |                     | 10 |

Note 1:

The molten pig iron of 1250°C was filled in a ladle (250 t) and added with the above mentioned desulfurizing agent as the molten pig iron being agitated by an impeller at 80 r.p.m.

Note 2:

The desulfurizing agent was added at the almost uniform rate of addition for 10 minutes. In all cases, the molten pig iron was agitated by an impeller for 16 minutes after the beginning of the addition.

15

| Inventive examples  | Desulfurizing agent | Size of desulfurizing agent | Mixing ratio of a gas generating substance and a reducing gas generating substance | Quantity of gas generating substance, added to carbide |  |
|---------------------|---------------------|-----------------------------|------------------------------------------------------------------------------------|--------------------------------------------------------|--|
| 15                  | calcium carbide     | 0.05 mm                     | lime stone : 90 %<br>polyester : 10                                                | 6 %                                                    |  |
| 16                  | "                   | 0.10                        | MgCO <sub>3</sub> : 80<br>plastic : 20                                             | 15                                                     |  |
| 17                  | "                   | 0.30                        | dolomite : 85<br>coke particle: 15                                                 | 11                                                     |  |
| 18                  | "                   | 0.01                        | polyester : 100                                                                    | 18                                                     |  |
| 19                  | "                   | 0.5                         | soda ash : 93<br>oil : 7                                                           |                                                        |  |
| Comparative example |                     |                             |                                                                                    |                                                        |  |
| 13                  | "                   | 0.01                        |                                                                                    |                                                        |  |

| Ratio of mixing in carrier gas (foaming gas) | Quantity of desulfurizing agent, added to molten pig iron | Rate of desulfurizing agent to be added | S in molten pig iron before desulfurization | S in molten pig iron after desulfurization | Reaction efficiency |
|----------------------------------------------|-----------------------------------------------------------|-----------------------------------------|---------------------------------------------|--------------------------------------------|---------------------|
| gas generating substance                     | rest: carrier gas                                         | kg/t-pig                                | kg/t-min.                                   |                                            |                     |
| 10                                           |                                                           | 2.5                                     | 0.1                                         | 0.03 %                                     | 0.01 % 19 %         |
| 30                                           | "                                                         | 2.7                                     | 0.2                                         | 0.04                                       | 0.015 23            |
| 50                                           | "                                                         | 4.1                                     | 0.3                                         | "                                          | 0.005 20            |
| 40                                           | "                                                         | 1.5                                     | 0.06                                        | "                                          | 0.02 30             |
| 25                                           | "                                                         | 1.0                                     | 0.5                                         | 0.03                                       | 0.01 40             |
|                                              |                                                           | 4.7                                     | 0.15                                        | 0.03                                       | 0.01 10             |

Note 1:

The molten pig iron of 1200°C was filled in a ladle (250 t) and the desulfurizing agent was blown in under the surface of the molten pig iron.

Note 2:

N<sub>2</sub> was used for the carrier gas (foaming gas).

| Inventive examples   | Quantity of carbide to be added | Petroleum substance          | Computed in terms of quantity of H <sub>2</sub> gas to be generated |
|----------------------|---------------------------------|------------------------------|---------------------------------------------------------------------|
| 20                   | 2.0 kg/t-pig                    | heavy oil<br>20 kg/t-carbide | 0.25 %                                                              |
| 21                   | 2.0                             | "<br>100                     | 1.00                                                                |
| 22                   | 2.2                             | tar<br>40                    | 0.3                                                                 |
| 23                   | 1.5                             | polyethylene<br>50           | 0.1                                                                 |
| 24                   | 1.3                             | propane(liquid)<br>80        | 0.5                                                                 |
| Comparative examples |                                 |                              |                                                                     |
| 14                   | 4.0                             |                              |                                                                     |
| 15                   | 4.0                             |                              |                                                                     |
| 16                   | 3.0                             |                              |                                                                     |

| Desulfurization method    | S in molten pig iron before desulfurization | S in molten pig iron after desulfurization | Desulfurization efficiency                                                                           |
|---------------------------|---------------------------------------------|--------------------------------------------|------------------------------------------------------------------------------------------------------|
|                           |                                             |                                            | $\frac{\text{CaC}_2 \text{ taking part in desulfurization reaction}}{\text{added CaC}_2} \times 100$ |
| addition with carrier gas | 0.028%                                      | 0.012                                      | 21.3%                                                                                                |
| "                         | 0.033                                       | 0.006                                      | 50.0                                                                                                 |
| "                         | 0.040                                       | 0.010                                      | 40.0                                                                                                 |
| agitation                 | 0.035                                       | 0.005                                      | 36.2                                                                                                 |
| "                         | 0.030                                       | 0.005                                      | 44.0                                                                                                 |
| addition with carrier gas | 0.028                                       | 0.011                                      | 10.8                                                                                                 |
| "                         | 0.040                                       | 0.020                                      | 13.3                                                                                                 |
| agitation                 | 0.030                                       | 0.011                                      | 17.0                                                                                                 |

## Note 1:

The addition with carrier gas, shown in the column "desulfurization method", means that a desulfurizing agent (calcium carbide) was carried with  $N_2$  gas, the carrier gas, to be added into the molten pig iron. The agitation shows that the molten pig iron is mechanically agitated by an impeller and added with a desulfurizing agent to further the contact with the molten pig iron.

## Note 2:

In the examples 20, 21 and 22, the petroleum substances and the desulfurizing agent (carbide) were added. The petroleum substance in the example 23 was pulverized an average of 0.1 mm and mixed with carbide to be added.

## Note 3:

The molten pig iron was desulfurized at 1320°C.

## What is claimed is:

1. A process for desulfurizing molten pig iron comprising introducing a mixture of calcium carbide and a solid material selected from the group consisting of polyethylene, vinyl chloride, and polyester, in a carrier gas, to the molten pig iron.

2. The process of claim 1 wherein a substance which generates carbon dioxide selected from the group consisting of limestone and magnesium carbonate is added

to the mixture.

3. The process of claim 2 wherein the ratio of amount of carbon dioxide generated to carrier gas is from 10 to 50 percent.

4. A process according to claim 1, in which the particle size of the calcium carbide is from 0.5 to 1.1 mm.

5. A process according to claim 1, in which  $H_2$ ,  $CH_4$ ,  $C_2H_2$ , or  $C_3H_8$  is contained in the carrier gas.

\* \* \* \* \*

35

40

45

50

55

60

65

**Notice of Adverse Decision in Interference**

In Interference No. 99,220, involving Patent No. 3,876,421, Y. Takemura, PROCESS FOR DESULFURIZATION OF MOLTEN PIG IRON, final judgment adverse to the patentee was rendered Oct. 12, 1976, as to claims 1 and 2.

*[Official Gazette February 1, 1977.]*